

## UNITED STATES PATENT OFFICE.

JOSEPH SEYER, OF HAWTHORNE, NEW JERSEY, ASSIGNOR TO STANDARD SILK DYEING CO., OF PATERSON, NEW JERSEY, A CORPORATION OF NEW JERSEY.

## WASHABLE SILK PIECE GOODS AND PROCESS OF DYEING IT.

No Drawing. Original application filed December 1, 1922, Serial No. 604,390. Divided and this application filed February 24, 1923, Serial No. 621,073. Renewed June 14, 1926.

This invention relates to a process of dyeing silk, and more particularly to a process of dyeing silk piece goods to produce washable silks in certain colors.

5 This application is a division of my original application Serial Number 604,390, filed December 1, 1922, patent Reissue No. 16,016 and this application particularly covers process #2 described in the original

10 application.

Said process #2 is applicable for the following colors:

|               |          |           |            |              |
|---------------|----------|-----------|------------|--------------|
| Turquoise     | Geranium | Beaver    | Strawberry | Emerald      |
| S. 6153       | S. 2035  | S. 3187   | S. 2185    | S. 5005      |
| 15 Hunter     | Myrtle   | Saxe blue | Electric   | Sapphire     |
| S. 5007       | S. 5067  | S. 6053   | S. 6055    | S. 6057      |
| Plum          | Prune    | Egg plant | Copenhagen | Delft        |
| S. 7187       | S. 7817  | S. 7905   | S. 6183    | S. 6185      |
| Slate         | Graphite | Smoke     | Taupe      | Castor       |
| S. 8067       | S. 8965  | S. 8935   | S. 8845    | S. 8843      |
| Raspberry     | National | Yale blue | Marine     | Cadet        |
| S. 2165       | S. 6005  | S. 6007   | S. 6083    | S. 6833      |
| 20 Regimental | Olive    | Evergreen | Cherry     | Ruby         |
| S. 6855       | S. 5485  | S. 5495   | S. 2063    | S. 2065      |
| Am. beauty    | Peacock  | Wisteria  | Magenta    | Fuchsia      |
| S. 2067       | S. 6505  | S. 7195   | S. 7285    | S. 7205      |
| Bottle green  | Violet   | Pansy     | Purple     | Old China    |
| S. 5827       | S. 7003  | S. 7005   | S. 7007    | S. 6184      |
| Japan blue    | Moss     | Carmine   | Bluebird   | Spring green |
| S. 6187       | S. 5483  | S. 2263   | S. 6065    | S. 5043      |
| Indiana       |          |           |            |              |
| S. 2064       |          |           |            |              |

25 The process is conducted as follows: Silk piece goods are dyed in a gum soap liquor, otherwise known as "boiled off liquor", acidulated with 2 lbs. 66° Bé. and 20 lbs. respectively of sulphuric and acetic acid, and the operation is begun by working the goods in this bath for 20 minutes, after which the dyestuffs such as basic, direct, or acid dyes are added to produce the shade desired as above. When the goods match the objective sample, there are added to the dye bath of 250 gallons liquor, 6 lbs. tannic acid



30 and the goods are worked for one hour continuously at a boil. They are then well washed and treated in a cold bath of water comprising two hundred fifty gallons with 4½ lbs. tartar emetic



for 40 minutes. After this they are well washed and then cleaned in a soap bath at 160° F. The treatment is now concluded by 50 washing well and acidulating.

In the above described process, basic, direct, and acid dyes are mentioned as being suitable to produce the desired shades, and it is desired to state here some examples of the dyes falling within these classes. As basic 55 dyes may be used brilliant green, Victoria blue, rhodamine (red), thioflavine T (yellow), and methyl violet 6B (blue) and 5R (red); as direct dyes, pontamine green BBX, diazoline dark brown, accordine seal 60 brown; as acid dyes, fast red, milling yellow, formyl violet, formyl blue, nigrosine. This list is illustrative, not exhaustive, as other dyes may be used according to their nature and shade. It is to be understood that where 65 I mention exact temperatures and exact working conditions, deviations may be made according to the particular circumstances and I mention such working conditions in an exact manner in order to set forth a preferred embodiment.

While the colors above listed may be produced by the use of various dyes and combinations of dyes, it is desired for the sake of specific examples, to mention dyes that 70 may be used. Turquoise and peacock are obtained with Victoria blue and brilliant green crystals; geranium, indiana, ruby, are obtained with rhodamine B, thioflavine T, and methyl violet 5R; slate, beaver, graphite, 75 smoke, taupe, and castor are obtained with pontamine green BX, diazoline dark scarlet, and chrysophenine G; strawberry is obtained with chlorantine violet BL and diazoline dark scarlet; emerald is obtained with 80 brilliant green crystals and thioflavine T; plum, hunter, and myrtle are obtained with methyl violet 5R, thioflavine T, Victoria 85 blue, and brilliant green; saxe blue, electric, sapphire, copenhagen, delft, Japan blue, old 90 China, are obtained with Victoria blue, methyl violet 5R, and brilliant green; prune and eggplant are obtained with methyl violet 6B plus the dyes for plum; raspberry is obtained with diazoline dark scarlet, ac- 95 cordine maroon, and chlorantine violet BL; national, Yale blue, and marine are obtained with Victoria blue, methyl violet 6B, rhodamine, and brilliant green; cadet and regimental are obtained with pontamine green 100

BX and diazoline dark scarlet; olive and evergreen are obtained with Victoria blue, thioflavine T, methyl violet 5R, and brilliant green; cherry and carmine are obtained with rhodamine B and thioflavine T; bottle green is obtained with pontamine green BX, chrysophenine G, methyl violet 6B, and brilliant green; violet, pansy, and purple are obtained with methyl violet 5R, and blue purple dye; American beauty, magenta, and fuchsia are obtained with rhodamine B, thioflavine T, and methyl violet 6B; wisteria is obtained with methyl violet 6B, brilliant green, rhodamine B, and thioflavine T; moss is obtained with Victoria blue, thioflavine T, methyl violet 5R, and brilliant green; bluebird is obtained with Victoria blue; and spring green is obtained with brilliant green and thioflavine T.

As a result of the above process there are produced varieties of dyed silk piece goods which are washable, that is, they may be washed in water containing soap at a temperature of 110° F. and they will, in most cases, stand 180° F. without suffering unevenness in shade or color, or distinct loss of color. In addition to the highly desirable quality of being washable, these piece silks have also the property of being washable without imparting any substantial amount of their color to the washing liquid, such as water or soap solution. These results have not hitherto been achieved with silk piece goods dyed in the colors and shades of colors above enumerated. They are also dyed evenly, that is, without irregularity in the color, or unevenness of shade. These results have not hitherto been achieved with silk piece goods and I have not only been able to attain these results in certain colors but have been able to extend them to all colors and shades thereof. The alizarine dyes, which are used for the production of fast colors in skein silk, are expensive and exist only in a limited number of shades. My new silk goods may be washed together with silk, cotton, artificial silk, wool, etc., without staining them, at a temperature of about 110° F. or higher. They also have excellent fastness to light and ironing. In the case of the present Process No. 2 they will contain a metallic mordant, such as antimony. My new piece silk goods have the properties enumerated in my aforesaid original application.

While my silk piece goods have been described as being of unmixed silk, it is also possible to manufacture mixed silk goods, such as silk and cotton, by the above described process. The colors above enumerated are those appearing in the Color Card of America issued by the The Textile Color Card Association of the United States, 5th Edition.

As many apparently widely different em-

bodiments of my invention may be made without departing from the spirit thereof, I do not intend to limit myself to any particular embodiment except as indicated in the following patent claims.

70

I claim:

1. Silk goods dyed in the piece to a deep color, and having the characteristics of fastness to washing in lukewarm soap water, and of evenness in color.

75

2. Silk goods dyed in the piece to a deep color, and having the characteristics of fastness to washing in lukewarm soap water, and of fastness to a hot iron.

3. Silk goods dyed in the piece to a deep color, and having the characteristics of fastness to washing in lukewarm soap water, and of not bleeding in an aqueous liquid.

80

4. Silk goods dyed in the piece to a deep color, and having the characteristics of fastness to washing in lukewarm soap water, evenness in color, and fastness to a hot iron.

85

5. Silk goods dyed in the piece to a deep color, and having the characteristics of fastness to washing in lukewarm soap water, evenness in color, fastness to a hot iron, and not bleeding in an aqueous liquid.

90

6. Silk goods dyed in the piece, and having the characteristics of fastness to washing in lukewarm soap water and evenness in color, and containing a metallic compound in the fibre.

95

7. Silk goods dyed in the piece, and having the characteristics of fastness to washing in lukewarm soap water, and evenness in color, and containing an antimony compound in the fibre.

100

8. Silk goods dyed in the piece to a deep color and having the characteristics of fastness to washing in lukewarm soap water, and evenness in color, and containing a metallic compound in the fibre.

105

9. Silk goods dyed in the piece to a deep color, and having the characteristics of fastness to washing in lukewarm soap water, and evenness in color, and containing an antimony compound in the fibre.

110

10. The process of dyeing silk piece goods to obtain a color fast to washing in lukewarm soap water, characterized by dyeing the goods and thereupon mordanting them in a hot liquor.

115

11. The process of dyeing silk piece goods to obtain a color fast to washing in lukewarm soap water, characterized by dyeing the goods in a hot soap liquor and thereupon mordanting them in a hot soap liquor.

120

12. The process of dyeing silk piece goods to obtain a color fast to washing in lukewarm soap water, characterized by dyeing the goods and thereupon mordanting them in a continuously boiling liquor.

125

13. The process of dyeing silk piece goods to obtain a color fast to washing in lukewarm soap water, characterized by dyeing

130

the goods and thereupon mordanting them in a continuously boiling gum soap liquor.

14. The process of dyeing silk piece goods to obtain a color fast to washing in luke-warm soap water, characterized by dyeing the goods and thereupon mordanting them with tannic acid in a continuously boiling liquor and treating them thereafter with tartar emetic.

15. The process of dyeing silk piece goods to obtain a color fast to washing in luke-warm soap water, characterized by dyeing the goods and thereupon mordanting them with tannic acid in a continuously boiling gum soap liquor and thereafter treating in a cold water bath with tartar emetic.

16. The process of treating silk piece goods comprising dyeing them in a continuously boiling liquor, and adding a mordanting agent to the boiling liquor.

17. The process of dyeing silk piece goods to obtain a color fast to washing in luke-warm soap water, characterized by dyeing the goods, thereupon mordanting them, and then cleansing with a hot soap solution.

18. The process of dyeing silk piece goods to obtain a color fast to washing in luke-warm soap water, characterized by dyeing the goods, thereupon mordanting them in a boiling soap liquor, and then cleansing with a hot soap liquor.

19. The process of treating silk piece goods comprising dyeing them in a continuously boiling gum soap liquor, and adding a mordanting agent to the boiling liquor.

20. The process of treating silk piece goods comprising dyeing them in a boiled off liquor, mordanting the dye and working the goods at a boil, washing, and cleaning in a soap water bath.

21. The process of treating silk piece goods comprising dyeing the goods to the desired shade in an acidulated, boiled off liquor, adding tannic acid and working the goods, washing, treating the goods with tartar emetic, washing, cleaning in a soap water bath, and washing and acidulating.

22. The process of treating silk piece goods comprising dyeing them in a boiled off liquor acidulated with an acid, the dye bath containing a dye, treating them with tannic acid, washing them, treating them in a cold water bath of two hundred fifty gallons with tartar emetic for 40 minutes, washing them, cleansing with soap water solution at 160° F., and washing and acidulating.

23. The process of treating silk piece goods comprising working the goods in a boiled off liquor, adding a dye to produce

the shade of color desired, adding tannic acid and working the goods at a high temperature, washing, treating the goods with tartar emetic, washing, cleaning in a soap water bath, and washing and acidulating. 65

24. The process of treating silk piece goods comprising working the goods in two hundred fifty gallons of gum soap liquor acidulated with an acid, adding a dye to produce the shade of color desired, adding tannic acid and working the goods for one hour at a boil, washing, treating the goods in a cold water bath of two hundred fifty gallons with tartar emetic for 40 minutes, washing, cleaning in a soap water bath at 75 160° F., and washing and acidulating.

25. The process of treating silk piece goods comprising dyeing them in a continuously boiling liquor, and thereupon mordanting them in the same boiling liquor. 80

26. The process of treating silk piece goods comprising dyeing them in a continuously boiling liquor and then adding tannic acid to the boiling liquor.

27. The process of dyeing silk to obtain a color fast to washing in lukewarm soap water characterized by dyeing it, and thereupon mordanting it in a boiling soap liquor. 85

28. The process of dyeing silk to obtain a color fast to washing in lukewarm soap water, characterized by dyeing it in a hot liquor, and thereupon mordanting it with tannic acid in a continuously boiling gum soap liquor. 90

29. The process of treating silk, comprising dyeing it in a continuously boiling liquor and then mordanting it in the same boiling liquor. 95

30. The process of treating silk, comprising dyeing it in a continuously boiling liquor and then adding a mordanting agent to the boiling liquor, and thereafter treating with tartar emetic. 100

31. The process of treating silk comprising dyeing it in a continuously boiling liquor, then mordanting it, and finally cleansing with a hot soap solution. 105

32. The process of treating silk comprising dyeing it, then mordanting the dye on the silk in a continuously boiling soap liquor, and thereafter cleansing with a hot soap solution. 110

33. The process of treating silk comprising dyeing it in a gum soap liquor and then mordanting it in the same liquor at a boiling temperature. 115

In testimony that I claim the foregoing, I have hereunto set my hand this 21st day of February, 1923.

JOSEPH SEYER.